



US006391155B1

(12) **United States Patent**  
Wurster et al.

(10) **Patent No.:** US 6,391,155 B1  
(45) **Date of Patent:** \*May 21, 2002

(54) **COATED WEB PRINTING PAPER SUITABLE  
FOR COLD-SET OFFSET PRINTING**

(75) Inventors: **Hartmut Wurster**, Friedberg;  
**Hans-Peter Hofmann**, Dachau, both of  
(DE)

(73) Assignee: **Haindl Papier GmbH**, Augsburg (DE)

(\*) Notice: Subject to any disclaimer, the term of this  
patent is extended or adjusted under 35  
U.S.C. 154(b) by 0 days.

This patent is subject to a terminal dis-  
claimer.

(21) Appl. No.: **09/655,723**

(22) Filed: **Sep. 5, 2000**

**Related U.S. Application Data**

(63) Continuation-in-part of application No. 09/169,010, filed on  
Oct. 9, 1998, now Pat. No. 6,197,155.

(30) **Foreign Application Priority Data**

Oct. 11, 1997 (DE) ..... 197 45 082

(51) **Int. Cl.**<sup>7</sup> ..... **D21H 27/00; D21H 17/04;**  
D21H 17/28; D21H 17/68

(52) **U.S. Cl.** ..... **162/135; 162/158; 162/181.1;**  
162/181.8; 162/175; 162/173; 428/340;  
428/341

(58) **Field of Search** ..... 162/135-137,  
162/158, 181.1-181.8, 175, 173; 427/391,  
361; 428/331, 537.5, 688, 446, 330, 340,  
341, 328; 106/465, 416, 20 R, 468, 464,  
463, 486, 474

(56)

**References Cited**

**U.S. PATENT DOCUMENTS**

|              |          |                       |           |
|--------------|----------|-----------------------|-----------|
| 4,820,554 A  | 4/1989   | Jones et al. ....     | 427/391   |
| 4,826,536 A  | 5/1989   | Raythatha et al. .... | 106/465   |
| 4,854,971 A  | 8/1989   | Gane et al. ....      | 106/286.5 |
| 4,943,349 A  | 7/1990   | Gomez ....            | 162/158   |
| 5,120,365 A  | 6/1992   | Kogler ....           | 106/415   |
| 5,423,911 A  | 6/1995   | Coutelle et al. ....  | 106/416   |
| 5,882,396 A  | 3/1999   | Hiorns ....           | 106/464   |
| 5,916,420 A  | * 6/1999 | Wurster et al. ....   | 162/137   |
| 6,197,155 B1 | * 3/2001 | Wurster et al. ....   | 162/135   |

**FOREIGN PATENT DOCUMENTS**

|    |            |        |
|----|------------|--------|
| DE | 4400609    | 7/1995 |
| EP | 0377983    | 7/1990 |
| EP | 0777014    | 6/1997 |
| EP | 0785307 A2 | 7/1997 |
| JP | 04057988 A | 2/1992 |

**OTHER PUBLICATIONS**

J. Stephenson, "Manufacture & Testing of Paper and Board", *McGraw-Hill Book Company, Inc.*, vol. 3, pp. 691, 1953.

\* cited by examiner

*Primary Examiner*—Jose Fortuna

(74) *Attorney, Agent, or Firm*—Smith, Gambrell, & Russell, LLP

(57) **ABSTRACT**

A lightweight, coated web printing paper is described which is suitable for use in the cold-set printing process, which has specific values for water penetration and ink absorption and has gloss values of at least 20% for a smoothness in the range of 200 to 600 sec. Bekk.

**20 Claims, No Drawings**

## COATED WEB PRINTING PAPER SUITABLE FOR COLD-SET OFFSET PRINTING

### RELATED U.S. APPLICATION DATA

The present application is a continuation-in-part application of U.S. patent application No. 09/169,010, filed Oct. 9, 1998 now Pat. No. 6,197,155, which is incorporated herein by reference in its entirety.

### BACKGROUND OF THE INVENTION

The invention relates to a coated web printing paper suitable for printing with cold-set offset printing ink.

If one commonly refers to offset printing, offset printing with heat-set printing inks is typically intended, and not the use of an offset process using cold-set inks. The cold-set process is predominantly used for the printing of newspapers on uncoated newsprint paper, and the printing presses used are therefore commonly referred to as newsprint printing presses.

The heat-set offset process, on the other hand, covers an entirely different field of application, and is, similar to the rotogravure process, predominantly used for high quality multi-color printing applications on coated, high-finish supercalendered papers up to the highest grades.

A patent which is believed to describe such conventional supercalendered papers suitable for heat-set offset printing is U.S. Pat. No. 4,820,554 to Jones et al. An object of the Jones et al. patent is to provide a chemically modified kaolin based pigment that shows enhanced gloss development during supercalendering of a paper coated with a coating formulation which contains this modified pigment. In order to demonstrate the improved gloss development, the patent includes a number of examples—such as Examples XVI, XVII and XVIII—in which certain base papers were coated with a coating formulation including various proportions of the modified kaolin, and the properties of the papers then tested. For comparison purposes, a coating formulation containing as pigment 100% Betagloss, a standard kaolin brand from E.C.C. America, was used.

The pigments used and the test papers prepared in the Jones et al. patent appear in all respects to be those typically used for conventional heat-set offset printing, and thus unsuited for the cold-set offset printing method. The example portion of the present application provides a comparison of the properties of the paper according to the claimed invention with that prepared according to the teachings of the Jones, et al. patent, demonstrating the clear differences between the papers according to the claimed invention and those prepared according to the teachings of the Jones et al. patent concerning suitability for the cold-set offset printing process.

It is understood by those skilled in the art that uncoated, common newsprint paper has a high receptivity for liquids, due to the absence of a paper coating. This is why it has been possible to use a printing ink which is absorbed quickly and therefore dries quickly, so that no additional energy in the form of heat or other radiation energy is necessary to assist printing ink drying. The newsprint printing presses are therefore designed accordingly.

Because newsprint presses remain idle for much of the day, there was a desire to use these presses for higher-quality printing applications during this idle time. Yet, conventional magazine grade coated papers designed for heat-set and rotogravure printing processes proved unsuitable for use on newsprint presses. There was therefore a need to provide a

commercially successful machine-coated paper which could be processed on newsprint presses in the speed range applied for the printing of uncoated newsprint.

A matte paper having generally suitable characteristics for cold-set offset printing is described in EP-A 0 785 307. As regards the need for enhanced cold-set paper qualities and the related problems, the introductory statements in this older document are helpful.

However, the web printing paper described in EP-A 0 785 307 is only of a so-called matte quality. It is explained in this document that to achieve the pressability and printability of a coated web printing paper in the cold-set offset process, special demands must be made on the paper regarding its wetting/water penetration behavior and its ink absorption speed. These are properties which at times are in turn considerably disadvantaged by a glazing on smoothness of from 1,000 to 1,600 sec. Bekk, as is necessary for producing typical smooth papers. For this reason, it was only possible according to this document to provide a coated matte quality paper suitable for the cold-set offset process. High smoothness and gloss, which indicate surface compaction, are thus generally detrimental to cold-set applications.

A high degree of advertising effectiveness is presently desired through the use of newspaper supplements, and only glossy paper can be considered for certain advertising orders. In the absence of cold-set-suitable glossy low weight coated (LWC) papers, these brochures are still printed via the conventional heat-set process as before. To enable the cold-set printer to take on such printing orders as well, the main point leading to the present invention was a desire to develop a glossy paper quality that closes this quality gap, and which can be pressed and printed without problems via the printing machine configurations that are typical in the newspaper printing domain (eight-tower and satellite printing machines). After such a paper quality has been established in the domain of mass-produced printing paper, economic aspects were also to be taken into consideration.

### OBJECTS OF THE INVENTION

It was therefore an object of the claimed invention to provide a coated web printing paper for the cold-set process that has sufficient gloss for more demanding printing products, in particular advertising supplements and the like, and which can be manufactured economically.

This technical problem is solved by the features of the claimed invention.

### DETAILED DESCRIPTION OF THE INVENTION

The matte paper described in EP-A-0 785 307 for the cold-set process, though not obtaining the gloss which is necessary according to the claimed invention, is indicative of papers which are suitable for cold-set offset printing. The paper according to this document is first of all characterized by its water absorbency, measured on the wetting angle of contact of a water drop or by determining the penetration behavior. A further important property of the paper, which may be dependent on the printing machine to a certain extent, however, is the ink absorption behavior of the paper.

It was indicated in EP-A-0 785 307, namely on page 12, lines 19–23, that the two aforementioned properties reciprocally determine each other to a certain extent, in such a way that a paper is also suitable for printing in the cold-set process if the values for the water absorption capacity and the ink absorption range in their opposite limit ranges, in such a way that in this case a certain compensation of the properties seems to take place.

It has also been determined that a glossy printing paper with cold-set suitability cannot be obtained by glazing to a high smoothness value as is otherwise typical for LWC papers.

Not only the combination of the two aforementioned properties, which appear essential for suitability in the cold-set process, is affected by this. In addition, the paper's pick-resistance, generally required for the offset process, is also reduced. This effect cannot be compensated for to a corresponding degree by additional binder in the coat, because the binder in turn influences the two basic values considered decisive for the cold-set process.

It has been determined that glazing to smoothness values of more than 1,000 sec. Bekk. of a basically cold-set-suitable printing paper destroys the cold-set suitability. Smoothnesses in the range of approximately 600 sec. Bekk. are still feasible for such uses, however. Acceptable gloss values can be attained according to the invention with smoothnesses as of 200 sec. Bekk. A preferred range is 300 to 400 sec. Bekk. The finishing of the paper with such a smoothness may already have reactions on the pressability and printability in the cold-set process, however.

But even a glazing to smoothnesses in the 600 sec. Bekk. range does not yet necessarily lead to a paper with a strived-for gloss which, measured according to Lehmann, should be at least roughly 20% at a 75° angle. The gloss for the indicated limited smoothness can be increased by the selection of suitable coating pigments. This selection is relatively stratified, however, such that it is difficult to individually indicate the coating pigment compositions leading to the success strived for. This is made even more difficult by the fact that different coating pigment compositions as a rule also require qualitatively and quantitatively different binder compositions/proportions, which in turn have a reaction on the basic values required for the cold-set suitability. The paper according to the invention is therefore defined by minimum gloss values in addition to the ranges for water absorbency, ink absorption and smoothness. Within the framework of the tests taken as a basis for the invention, basic selection criteria were determined that lead to the strived-for success and provide the expert a sufficient lesson as to how one shall proceed. These selection criteria are included in subclaims. In addition, the added examples of execution contain concrete details as to how a paper according to the invention can be produced.

The possible and preferred limits for the smoothness values to be adhered to were already indicated. Water absorption according to the Emco test should be situated in the 85–25% range after one second, preferably in the 70–30% range. The ink absorption test should yield a value of 1.1 to 0.25, preferably a value of 0.8 to 0.3. Gloss measured according to Lehmann at 75° should be at least 20%, but preferably between 25 and 55%, to yield a glossy appearance of the paper that is commonly considered sufficient.

The testing methods used, in particular the method of gloss measuring, are explained in further detail below. The penetration test according to Emco and the ink absorption test are defined as already described in EP-A-0 785 307.

The paper described in this case must also have a pick-resistance sufficient for the offset process. This pick-resistance is determined and qualitatively assessed in typical manner. In this regard as well, the statements in EP-A-0 785 307 are referred to.

Fine-particle pigments in the coat composition generally accelerate printing ink drying (shortening of the ink absorp-

tion time, expressed by a lower densitometer value) and water absorption. With the selection and/or mixture of the pigment grading, the expert therefore has the ability, according to the invention, to influence both values. If it is possible with a specific printing machine arrangement to press a paper that has very rapid ink absorption times, highly active synthetic binder is preferably chosen as binder for the coater, in connection with polyvinyl alcohol to the extent possible. The binder for such a coater can thus consist of 6–12% synthetic binder and from 1% to 4% PVA in relation to coating pigment. If a longer ink absorption time is required with the same water absorbency, this can be achieved by additional binders in the coat recipe, for example by adding 0.5 to 1.5% carboxyl methyl cellulose (CMC), depending on the composition of the coating pigment. If the binder is given additional starch, in the range of roughly 6–10 weight percent, for delaying the ink absorption time, this may also have a reducing influence on water absorbency.

Beyond the binder content and mixture also influenced by the fineness of the gloss-developing pigments used, the necessarily high water absorbency, the desired printing ink drying time and a good coat setting should be taken into account. In addition, it should be taken into consideration that the paper gloss values decrease as the binder content increases. Altogether, the binder content in the coater should not exceed 18 weight percent in relation to coating pigment. The higher values below this limit come into consideration when starch and/or CMC are used in addition to synthetic binders.

In paper coating, in general the following types of binder are used, in order of decreasing binding action: plastic dispersions (e.g. styrol-butadiene, acrylate, styrol-acrylate), PVA, protein or casein, and starch. Highly active binders are the aforementioned plastic dispersions, also in combination with PVA. For certain binders, the adding of a cross-linking agent may be required.

If work is only done with highly active, synthetic binders in certain cases of application, the total binder proportion may be below 16 weight percent in relation to coating pigment, preferably even below 14 weight percent. Besides its binding force, PVA also has the property of being absorbed irreversibly on surfaces that have a relatively inert reaction capacity, as is true in the case of the calcium carbonate used within the framework of the invention.

The binder proportions may be as follows:

|                |                     |
|----------------|---------------------|
| plastic binder | 3–10 weight percent |
| PVA            | 0–5 weight percent  |
| protein        | 0–5 weight percent  |
| starch         | 0–10 weight percent |
| CMC            | 0–2 weight percent  |

In the case of the classic coating pigments, after the gloss development increases, the ink absorption time decreases and the binder requirement (higher pigment surface) increases as the degree of fineness increases, the pigments must be selected and composed according to the requirements of the invention. Pigments with a higher degree of paper gloss development are

- a) kaoline qualities with high grain fineness (94–100% <2  $\mu\text{m}$ ), such as Amazon 88, Euroclay FC, Hydraglass E, etc.
- b) Natural, ground calcium carbonates (GCC) with a fineness of 98±5% <2  $\mu\text{m}$ , such as Carbilux, Setacarb HG and M, Hydracarb CCM, etc.

c) Synthetic, precipitated calcium carbonates (PCC) with a mean particle size of preferably 0.5–1.0  $\mu\text{m}$ . In this product group, preferably products with rhombohedral crystal shape are advisable because of the more advantageous binder requirement. Needle-shaped PCC qualities, such as aragonites and scalenohedric particles require high binder proportions for setting on the body paper and lead to extremely short ink absorption times. The needle-shaped pigments proposed in EP-B-0 377 983 have, according to the presentation therein, a high oil adsorption, which is roughly synonymous with a high binder adsorption.

d) Synthetic pigments:

This product group indeed increases paper gloss development, but reduces the wet pick-resistance and increases coat costs.

It has proven advantageous to work with pigment blends, whereby the advantages of the individual pigments can be made use of and the disadvantages can be reduced. For this reason, for controlling the coat quality, the use of laminar pigments with lower grain fineness can also be advantageous. Thus, for example, by also using a kaoline with laminar particles, of the SPS quality of the company ECC with a fineness of 80%  $<2 \mu\text{m}$  and a particle shape factor of 21, the coating hold-out of color systems containing a high degree of fine particles is improved, whereby gloss development increases and ink absorption time is prolonged.

In addition, the coaters used may contain typical additives, such as up to 1.5 weight percent melamine formaldehyde resin as a wet-strength agent, up to 0.4% carboxyl methyl cellulose (CMC) as a solution, optical lightener and/or chemicals for pH value setting, such as NaOII.

The coaters according to the invention are processed in aqueous slurry with solid contents of 30–65 weight percent of mathematical dry mass. As application processes, scraper application processes such as Inverted Blade, Jet Flow as well as roller application devices such as the Massey coater and also film presses such as the Jagenberg film press, the Speedsizer or the Metering Size Press from Beloit come into consideration. In the paper according to the invention it is understood one or the other of the application methods can lead to a better result, under certain conditions. As is well-known, scraper coating processes equalize the paper surface and therefore locally lead to coat application of different thicknesses, while roller coating devices rather produce a uniform coat application, which can be positive for the ink absorption behavior under certain circumstances. A gentle coat drying can also be significant, so that undesired binder migration phenomena do not worsen the strived-for uniform micro-capillarity of the coat application.

In the case of single-coated papers, according to the invention, mathematical dry coating quantities with a mass surface density of more than 4 g/m<sup>2</sup> and side are applied on the base paper. Mass surface densities of 6–12 g/m<sup>2</sup> and side, typically approx. 7 g/m<sup>2</sup> and side, are preferred.

The invention is not limited to single-coated paper, however. It is also applicable to double-coated paper. Double coats have a mass surface density of at least 15 g/m<sup>2</sup> and side, typically 20 g/m<sup>2</sup> and side, in connection with which the coating mass is spread roughly uniformly on both coat applications. The cover coat is obviously important for the paper's properties according to the invention. If a coat application is discussed within the framework of this description without it being designated in more detail, for single-coated papers the sole coat application is generally meant and for double-coated papers the cover coat is generally meant. The pre-coat in the case of double-coating is

always expressly designated as such within the framework of this description. The pre-coat may have a composition differing from the cover coat.

It may be useful to pre-smooth the base paper before application of the single coat or the pre-coat, for example in a machine-glazer at the end of the paper machine, which may also be equipped with a so-called soft-nip.

The invention is not limited to the use of a specific base paper, however. Thus, wood-free as well as wood-containing base papers and those with a considerable portion of processed, used paper fibers can be used. Thus, for example, a wood-free base paper is suitable whose furnish for the paper production contains in mathematical dry portions roughly 78% cellulose, roughly 20% mineral filler, roughly 1% starch and roughly 1% other adjuvants.

However, wood-containing base papers that additionally contain a portion of processed used-paper fibers are preferred for reasons of cost. In addition, wood-containing base papers as a rule also have printing advantages, for example greater opacity. The fibrous furnish for a wood-containing and used-paper-containing base paper can consist, for example, in relation to mathematical dry total fibrous substance, of roughly 20% cellulose, 20% wood pulp and 60% used-paper substance. In relation to the fibrous substance, the furnish may also contain up to roughly 50% mineral filler, which corresponds roughly to a  $\frac{1}{3}$  portion of the substance composition. As is well-known, this filler quantity does not remain completely in the paper in the production process, but rather partially makes its way into the process water.

Within the framework of this description, when wood pulps are spoken of as a fibrous component, these may be all such substances that are typically understood in paper technology with this expression, namely wood pulp, thermomechanical wood pulp (TMV), chemico-thermo-mechanical wood pulp (CTMP), etc.

A further important precondition for an acceptable printing result when printing on a paper with cold-set printing inks, in addition to a satisfactory drying of the printing inks, is the dimensional stability of the paper. Since water also penetrates into the base paper carrying the coat during the absorption of the cold-set printing inks, this has an effect on the fiber's bond to each other and thereby influences the dimensional stability of the paper. This influence is greater compared to normal newspaper-printing natural paper, because with a coated paper with comparable mass surface density the base paper as body paper for the coat only receives a correspondingly smaller mass portion, that is, the base paper is thinner. The dimensional stability of a paper under the influence of moisture can be improved by additives, for example starch. Thus, it is typical to add roughly 0.5 % to 2.0% starch to a base paper furnish. For papers that are produced on open endless wire paper-making machines or on so-called hybrid-formers in which an upper dewatering screen is combined with the endless wire only after successful sheet formation on it and that, as a result of this production process, have a relatively favorable fiber orientation relation, namely a crosswise-to-lengthwise ratio of roughly 1:2 up to a maximum of 1:2.5, the dimensional stability for their use in the cold-set printing process is possibly already sufficient without starch being added to the base paper at all. Due to the fiber orientation mainly in the production direction, that is in the longitudinal direction of the paper, the lack in dimensional stability consist essentially in a crosswise contraction, which is further increased by the pull of the paper web in the processing machine.

Mass-production printing papers are economically produced nowadays mainly on very fast-running paper machines which use exclusively so-called gap-formers

according to the current state of the art. With these gap-formers the sheets are formed in the convergence gap of two screens. With papers produced on such modern machines, the crosswise-to-lengthwise ratio of the fiber orientation is substantially poorer and ranges from roughly 1:3 to 1:4. This results in a substantially lower crosswise stability of such papers. The dimensional stability of base papers produced on gap-formers can be sufficiently positively influenced if more than 1%, to a maximum of 2%, typically roughly 1.5%, starch is added to the base paper furnish. The use of a highly cationic starch is preferred. Its effect is that when adding roughly 1.5% of this starch to the furnish, roughly 1.4% is found in the base paper, which indicates a surprisingly high retention of the starch during sheet formation, without the greater starch additive quantities remaining in the furnish without substantial effect on the base paper and at best increasing the waste-water load and the costs.

Since the paper according to the invention is first and foremost intended to cover the LWC range in the cold-set process, the mass surface densities of the finished paper are in the 40–80 g/m<sup>2</sup> range; masses of 54 and 60 g/m<sup>2</sup> are preferred.

The typical method for producing conventional glossy paper includes a further work step, glazing, after the coating process. This mechanical surface treatment is carried out for conventional LWC papers on a 12-roller calender under high pressure (up to 350 KN/m) and at high temperatures (up to 100° C.). In this procedure, the paper is highly compressed, whereby the surface smoothness increases and the volume decreases, effects that are contrary to the cold-set process quality requirements. To adhere to the quality data required for this domain of paper use according to the invention, only a light glazing is possible, for example 50 N/mm, via which the required gloss development is nevertheless achieved. Bekk smoothness values of 200, in particular 300 to not more than 600 sec. where possible, still display the required micro-capillarity via which a high degree of water penetration is ensured and gloss values in the 20–50% range can be obtained.

The production according to the invention of a paper with typically sufficient gloss but relatively little glazing and correspondingly low smoothness leads to a printing paper which, in addition to its cold-set suitability, has the following advantages compared to highly-glazed, glossy papers:

- greater specific volume
- greater stiffness
- greater dimensional stability, and thus improved passage preservation
- greater track stability during pressing
- less loss of lightness and whiteness
- less fiber mottling
- greater opacity.

In addition to the classic super-calender, in which not all roller nips are necessary for setting these low surface smoothnesses, other on-line and off-line smoothing aggregates are suitable for paper finishing, such as soft and Janus calenders.

Unless otherwise indicated in this description, percentages, even if this is not expressly mentioned, are always to be understood as weight percentages. Furthermore, unless otherwise specifically indicated, the percent quantities as well as other quantities always relate to the mathematical dry component. In this connection, the indication "otro" ("o-dry") relates to an oven-dry condition.

For measuring the immediate water absorption and/or penetration of a paper sample, the Dynamic penetration measuring apparatus DPM 27 of the company Emco Elektronische Mess- und Steuerungstechnik GmbH in 04347 Leipzig, Gorkistrasse 31, is used. The testing method is

based on this company's equipment description and operating instructions at the Mar. 13, 1995 status. The drop in the ultrasonic transmission value is measured starting from the measured value of the non-impregnated sample, which is equated with 100%, over the time. At the given time the measured value is indicated as a percentage of the initial value, which is equated with 100%. Basically speaking, this is a matter of a dynamic test in which a curve of the transmission drop is plotted over the time. This curve first drops steeply, then turns up and, at measuring times above 6 sec., approaches more or less asymptotically a specific transmission value. For the behavior of the paper, essentially the water absorption in the first moment is decisive, which is why the measured values after a time of 1 sec. are indicated for the purposes of this description. But the measured values after 3 sec. also have a certain significance for the evaluation; a time at which the steep curve drop swings approximately into the horizontal and a certain saturation point thus results. This testing method is designated in the following as an Emco test and the values are indicated in percentages (percent residual transmission, starting from 100%).

For determining the ink absorption, an absorption test, modified in the patent applicant's company and using the Dr. Dürner system multi-purpose sample printing machine of the company Prüfbau Dr.-Ing. Herbert Düner, Peissenberg, is used. In the ink absorption test, under defined conditions a sample print is produced with a standard printing ink, which is brought into contact under pressure with a counter-paper after a defined period of time. The printing ink intensity printed on the counter-paper is measured with a densitometer. In detail, during the counterpressure test, also designated as a blotting test or absorption test, a defined quantity of printing ink is applied on a strip of paper which is then rolled on section by section with a counter sample strip at predetermined intervals. The quantities of ink released on the counter sample strips are determined optically and allow conclusions as to the ink absorption behavior and the stacking behavior of the sample strip.

Details of the test execution can be seen in a thorough description for the multi-purpose sample printing machine of the company Prüfbau Dr. Ing. Herbert Dürner, Aich 17–23, D-82380 Peissenberg/Munich, of Sep. 26, 1972, in particular under 10.5 and 14.2.

Accordingly, for coated papers an inking supply of 0.3 cm<sup>3</sup>, a distribution time of 30 sec. in the inking unit and 30 sec. for the printing form are recommended. The contact pressure for the pressing and counterpressure should each be 200 N/cm, that is, 800 N for a printing form width of 4 cm. The absorption test ink no. 52 0068 of the Michael Huber ink factories in Munich should be used. The counterpressure should be carried out after 30, 60, 120 and 240 sec. As printing speed, 0.5 m/sec. is recommended. A standard paper with the designation APCO II/II of the Scheufelen company should be used as the sample printing paper.

In the present case, the tests were conducted at double printing speed and otherwise with the indicated values. The ink transfers onto the counter sample strip were evaluated that were attained after 30 sec. of counterpressure.

For measuring the gloss, the gloss measuring apparatus LGDL-02 Lab of the company Lehmann, Mess- und Regeltechnik in Biel, Switzerland, is used. The gloss measuring head LGML-02 for labs with an irradiation and re-radiation angle of 75° is used. The testing standards used for the gloss measuring are E DIN 54502 test of paper and cardboard, gloss evaluation of level paper and cardboard surfaces with the help of reflectometer values and Zellcheming specification V/22/72 test of paper, cardboard and pasteboard; measurement of the gloss.

Below are a few examples of execution.

## EXAMPLES

On a fast-running paper machine with a double screen former (gap former) a base paper was produced from the following furnish at a machine speed of roughly 1,300 m/min:

| base paper furnish                        |                         |
|-------------------------------------------|-------------------------|
| wood pulp                                 | 12.3%                   |
| cellulose                                 | 13.0%                   |
| used paper                                | 40.0%                   |
| filler                                    | 33.0%                   |
| highly cationic starch                    | 1.5%                    |
| retention agent                           | 0.2%                    |
| 100%                                      |                         |
| testing data of the base paper            |                         |
| mass surface density                      | 39.9 g/m <sup>2</sup>   |
| filler portion                            | 14.9%                   |
| braking load lengthwise                   | 42.0 N                  |
| braking load crosswise                    | 11.7 N                  |
| fiber orientation crosswise to lengthwise | 1:3.5                   |
| lightness                                 | 73.0%                   |
| volume                                    | 1.52 cm <sup>3</sup> /g |

Various coating tests were conducted with the base paper according to this example.

The test data reproduced in the following are those of a coating test with a coater with high kaoline content and those of a coating test with a coater that contained a rhombohedral, precipitated calcium carbonate as pigment. In the following table, there are details for both coating tests on the coater absorption, coat application and paper testing results.

| Coater recipe:<br>Pigments        | FG<br>[solid contents] | High kaoline<br>coater | High PCC<br>coater |
|-----------------------------------|------------------------|------------------------|--------------------|
| Rhomb. coating<br>(MPS 0.5 µm)    | 72%                    |                        | 100                |
| Amazon 88                         | 74%                    | 50                     |                    |
| SPS                               | 66%                    | 50                     |                    |
| <u>Binder:</u>                    |                        |                        |                    |
| Low-viscosity PVA                 | 20%                    | 2.0                    | 2.0                |
| Plastic binder                    | 50%                    | 7.0                    | 7.0                |
| Starch                            | 23%                    | 6.0                    | 6.0                |
| Optic lightener                   | 100%                   | 1.3                    | 1.3                |
| Cross-linking agent<br>(MF-resin) | 73%                    | 1.3                    | 1.3                |
| Synth. thickener                  | 25%                    | —                      | 0.2                |
| Coat weight:                      | g/m <sup>2</sup>       | 7.0                    | 6.9                |
| Moisture                          | %                      | 5.5                    | 5.6                |

| Paper testing results:               | High kaoline<br>coater | High PCC<br>coater |      |
|--------------------------------------|------------------------|--------------------|------|
| Mass surface density                 | g/m <sup>2</sup>       | 54.0               | 54.0 |
| Smoothness according<br>to Bekk      | sec.                   | 500                | 510  |
| Gloss 75° according<br>to Lehmann    | %                      | 41                 | 35   |
| Lightness                            | %                      | 74.9               | 76.4 |
| Whiteness with UV                    | %                      | 77.3               | 81.9 |
| Opacity                              | %                      | 92.1               | 91.5 |
| Ink absorption time<br>after 30 sec. | 0.4                    | 0.3                |      |

-continued

| 5  | Paper testing results:                                   | High kaoline<br>coater | High PCC<br>coater |
|----|----------------------------------------------------------|------------------------|--------------------|
| 10 | Wet pick-resistance<br>(1 = very good,<br>6 = very poor) | 2                      | 2                  |
| 15 | Emco measurement<br>after 1 sec.                         | %                      | 48 51              |

In the text column of the table, for the coater recipe for the individual components, the respective solid contents of the products are indicated on the right under the heading "FG". In addition, the text column contains on the right the measuring units for the measured values. In the value columns, in each case mathematical dry portions are indicated for the coater absorption. In addition to the coating pigments used for the tests, the following details are also provided:

## 20 Amazon 88

This is a matter of a kaoline for paper coating purposes of the company Cadam, Monte Dourado, Brazil, distributed by the company Kaoline International, NL-3447 Gv Woerolen, with a fineness of 96% <2 µm. The wet screen residues of particles >95 µm amount to 0.0035%. The whiteness level according to ISO 2740 is 86%.

## SPS

This quality is a kaoline with laminar particles of the company ECC International.

30 The shape factor of this pigment is 21, the degree of fineness is 80% of the particles <2 µm and 66% <1 µm. Rhomb. Coating (MPS 0.5 µm)

This pigment is a precipitated calcium carbonate with rhombohedral crystal structure of the company Faxe Kalk, DK-1017 Copenhagen K. The pigment has a fineness of 0.5 µm.

35 The test results show that with intentionally set smoothnesses of roughly 500 sec. Bekk, gloss values of 41% were achieved for the coater with high kaoline content and 35% for the coater with PCC. The water absorption measurement according to the Emco test was 48 and, respectively, 51%, and is thereby within the preferred range. The same applies to the ink absorption test with values of 0.4 and, respectively, 0.3.

40 The pick-resistance was to be considered good with the note 2. When using less smoothing with the same papers which led to smoothness values of roughly 250 sec. Bekk, no sufficient gloss values were able to be obtained with the coat compositions used. With an additive of 10% synthetic pigment to the coating pigments, a somewhat greater gloss was indeed able to be achieved, but the wet pick-resistance as the measure for offset suitability decreased, however.

45 When glazing a cold-set-suitable matte paper with 100% ground calcium carbonate as coating pigment, no sufficient gloss was able to be obtained with glazing to a smoothness of 500 sec. Bekk. The gloss was roughly only 18%. The opacity of the two test papers with values in the 92% range corresponds roughly to the opacity of a comparable matte paper and is thus to be considered very good.

55 A further experimental example was conducted, in which a paper was made by the process according to the claimed invention, and was compared with a paper made according to a reference already mentioned discussed, U.S. Pat. No. 4,820,554, to Jones et al. A comparison of the properties is instructive as to the differences between the paper according to the claimed invention and conventional glossy paper suitable for heat-set offset printing.

60 The object of the Jones et al. patent was to provide a chemically modified kaolin-based pigment which shows

enhanced gloss development during supercalendering of a paper coated with a coating formulation containing this modified pigment. The patent clearly does not relate to cold-set offset printing, and there is no suggestion that the paper prepared according to that patent would be useful for this purpose. An examination of a paper made according to the process taught in that patent bears further evidence that the paper is not suited for cold-set offset printing.

In Example XVI of the Jones, et al. patent, at column 18, lines 54–58, calendering conditions are recited to which apparently all of the test papers were subjected. The patent explains that the test papers were calendered for 10 nips at 1500 p.s.i. and a temperature of 150° F. The finished test papers were then tested for various gloss and printability properties.

While the patent recites calendering conditions in which a pressure of 1500 p.s.i. is used, there is some doubt whether the correct units were indicated. This is especially so since the gloss values obtained (presumably determined according to TAPPI with a Hunter apparatus) clearly indicate that the test papers described in the patent were subjected to full calendering in order to obtain a high gloss finish, as is common with supercalendered magazine papers to be printed by the heat-set offset or rotogravure printing methods. Table VI of Example XVI and FIG. 5 of the patent are noted, wherein it is shown that even with the Betagloss reference pigment a gloss value of 51% is obtained. It is noted that such supercalendered papers are unsuited for the cold-set offset printing method.

Concerning the recitation in the Jones et al. patent of a pressure of 1500 p.s.i., perhaps an error in the pressure units has occurred. Concerning the recitation in the Jones et al. patent of a calendering of 10 nips, the patent does not indicate whether a calender stack with 10 nips was intended, or whether the paper was simply passed 10 times through the single nip of a pilot plant or laboratory calender. This reflects also, of course, on the pressure measurement. There is likewise no indication of the calendering speed or the nature of the calender rolls.

Typically, calender pressure is cited in force per unit length of nip width, such as pounds per linear inch (p.l.i.) or N/mm. The calender pressure is typically not expressed in surface area units, since the actual contact area in a roll nip is difficult to determine, and will vary based on the pressure applied to the nip. In this regard, applicants refer to the textbook from Stephenson, "Pulp and Paper Manufacture," Vol. 3, "Manufacture & Testing of Paper and Board," McGraw-Hill Book Company, 1953, page 691, the disclosure of which is incorporated herein by reference, in which it is explained that "Machine-coated papers having a surface coated with various percentages of pigment coating ranging in weight from about 8 to 30 per cent, used for magazines, periodicals, catalogues, for reproduction of halftones, are being supered at nip pressures ranging from 1000 to 2000 lb. per linear inch of width on stacks having from 10 to 12 rolls, half of which are made of medium-hard-filled rolls and operated at speeds of 1600 to 1800 f.p.m." Applicants note that the pounds per square inch cited in the Jones et al. patent is a fairly uncommon unit, and that there is therefore reason to believe that the citation in the Jones, et al. patent is in error in that it should read 1500 p.l.i. instead of 1500 p.s.i.

Assuming a corrected value of 1500 p.l.i., the recited calendering conditions would fit those mentioned by Stephenson, 1500 p.l.i. being the mean value of the cited range of 1000 to 2000 p.l.i., and 10 nips being within the range of the 10 to 12 rolls recited in Stephenson.

The opinion of an expert was sought concerning this issue, and it was determined that several interpretations were possible. The first is that the pressure given described the pressure load on the cylinder of the hydraulic load system of the calender stack. If this first interpretation is correct, then

nothing further can be determined of the conditions used, since the pressure values would mean nothing as long as no piston diameters were given from which the actual load force could be calculated.

A second interpretation is that the 1500 p.s.i. refers to an assumed actual nip pressure. If this is the case, then the actual nip pressure under load would equal under usual nip width conditions a linear load of approximately 50 N/mm. Such low linear nip loads would not be realizable in a 10 nip/11 rolls calender stack because the roll weights alone would amount already to a nip load of about 100–200 N/mm. Low weight coated (LWC) papers with a gloss in the range of 50–60% are nowadays usually supercalendered with nip loads of some 300 N/mm.

A third interpretation is that the pressure of 1500 p.s.i. refers to the actual nip pressure determined from nip width measurements in a 1 nip/2 roll pilot plant calender for which a uniform nip pressure may be assumed, and that the test papers were passed ten times through the same nip. This would be the most slight conditions to be interpreted from the information given in the Jones et al. patent. It should be explained that in a multi-roll calender stack the nip pressure increases from top to bottom for reasons of the combined roll weights. In a single-pass pilot calender this is not the case. The nip load may therefore be pre-selected for the one and only nip.

Using the most slight calendering conditions of the three possible interpretations of the Jones et al. patent, Example XVI of the patent was, to the extent possible, reproduced. Because the particular pigment grades cited in the patent were not available, it was decided that the test be performed using the comparison pigment used in that patent, the Betagloss quality, which in any event rendered the lowest gloss values in the example.

It was determined that the former supplier of the Betagloss pigment, E.C.C. America, Inc., is in some way succeeded by the Imerys company, and some of the former brand names have been discontinued. However, inquiries at Imerys have confirmed that the present kaolin quality "Premier Slurry" is directly comparable to the former Betagloss brand. Thus, the "Premier Slurry" brand of Imerys was used for the reproduction tests.

From "Premier Slurry" kaolin, a 62% solids coating formulation was prepared in accordance with example XVI, column 18, line 17–25 of the Jones et al. patent, comprising:

100 parts kaolin Premier Slurry, calculated on a dry basis  
by weight,  
7 parts starch  
7 parts synthetic binder  
1.4 parts melamin-formaldehyde resin  
0.5 parts calcium stearate

As base stock for coating a publication grade base, stock generally corresponding to Table VI of the Jones et al. patent was used, but with a 49.4 g/m<sup>2</sup> basis weight, as a 43.8 g/m<sup>2</sup> version was not available. A coating of 8 g/m<sup>2</sup> was applied to the lower wire side of the paper, at a speed of 1500 ft/min., by a Cylindrical Laboratory Coater which is comparable to the Helicoater referred to in the Jones, et al. patent.

The coated paper was then calendered in one of two ways:

- according to the conditions of the Jones, et al. patent, as set forth above, i.e., 10 nip passes at a nip pressure of 50 N/mm (comparable to 1500 p.s.i.) at a temperature of 66° C. (equaling 150° F.) at a speed of 10 mn/min.;
- in a way as to render smoothness and gloss values as defined in claim I of the subject patent application, i.e., with one nip pass at a nip pressure of 47 N/mm at room-temperature at a speed of 10 in/min.

The comparison results are shown in the following table:

| Paper properties    | Calendering conditions |                   |
|---------------------|------------------------|-------------------|
|                     | Jones, et al. patent   | Second test paper |
| Smoothness Bekk sec | 1410                   | 290               |
| Gloss, Lehmann %    | 65                     | 38                |
| Emco Test 1 sec %   | 86                     | 83                |
| Ink absorption      | 0.19                   | 0.12              |

Under the assumed calendering conditions of the Jones, et al. patent, even with a nip load of only 50 N/mm, no gloss values below 60% could be obtained with 10 nip passes. The resultant smoothness of 1410 sec Bekk is beyond any suitability for cold-set offset printing. Consequently, also the two properties indicating coldest application, the Emco test and the ink absorption are out of the range of claim 1 of the application.

Thus, the paper re-produced from the Jones et al. patent, even with only the standard coating clay, does not meet any of the properties claimed in claim 1 of the present applications. Applicants note also that the second test paper, produced so as to obtain smoothness and gloss values as defined in claim 1 of the subject patent application, is still out of range as far as the coldset properties, i.e., the Emco test and the ink absorption, are concerned.

Further variations and modifications will be apparent to those skilled in the art from the foregoing, and are intended to be encompassed by the claims appended hereto.

We claim:

1. A glossy, coated web printing paper for use with cold-set inks in a cold-set offset printing process, comprising:
  - a base paper, comprised of paper fiber, and a mineral filler; and
  - a coat application, comprised of coating pigment, and binder,
 wherein said paper exhibits
  - a value in an Emco penetration test after one second of from 25 to 80%,
  - a value in an ink absorption test of from 0.25 to 1.1,
  - a smoothness value according to Bekk of from 200 to 600 sec., and
  - a gloss value measured with a Lehmann apparatus at 75° of 20% or more.
2. The printing paper according to claim 1, wherein the value of said Emco penetration test is from 30 to 70%, the value of said ink absorption test is from 0.3 to 0.8, and the smoothness value according to Bekk is from 300–400 sec.
3. The printing paper according to claim 1, wherein the gloss value is from 25 to 55%.
4. The printing paper according to claim 1, wherein said coating pigment comprises particles in which 93% are smaller than 2  $\mu\text{m}$ .
5. The printing paper according to claim 1, wherein the coating pigment comprises at least one member selected from the group consisting of
  - kaoline with a grain fineness wherein 94 to 100% of said grains are less than 2  $\mu\text{m}$ ,
  - natural, ground calcium carbonate with a grain fineness wherein 93 to 100% of said grains are less than 2  $\mu\text{m}$ ,

synthetic, precipitated calcium carbonate with a mean particle size of from 0.5 to 1.0  $\mu\text{m}$ , and synthetic pigment.

6. The printing paper according to claim 5, wherein said synthetic, precipitated calcium carbonate is a rhombohedral crystal shape.
7. The printing paper according to claim 5, wherein said coating pigment comprises laminar particles in which 80% are less than 2  $\mu\text{m}$ .
8. The printing paper according to claim 1, wherein said binder comprises a synthetic binder which contains starch, and wherein a binder content of said coat application is less than 18 weight percent starch-containing binder, in relation to said coating pigment.
9. The printing paper according to claim 1, wherein said binder comprises a synthetic binder without starch, and wherein a binder content of said coat application is less than 16 weight percent starch-free binder, in relation to said coating pigment.
10. The printing paper according to claim 1, wherein the binder content of said coat application is less than 14 weight percent, in relation to said coating pigment.
11. The printing paper according to claim 1, wherein said binder of said coat application comprises 6–10 weight percent synthetic binder and 1–4 weight percent PVA, in relation to coating pigment.
12. The printing paper according to claim 1, wherein said binder of said coat application, as a weight percent of said coat application, comprises:
  - 30 3–10 weight percent plastic binder,
  - 0–5 weight percent PVA,
  - 0–5 weight percent protein,
  - 0–10 weight percent starch, and
  - 35 0–2 weight percent carboxyl methyl cellulose.
13. The printing paper according to claim 1, wherein said coat application has a mass surface density for single-coated papers of more than 4 g/m<sup>2</sup> and side.
14. The printing paper according to claim 13, wherein said mass surface density for single-coated papers is 7–12 g/m<sup>2</sup> and side.
15. The printing paper according to claim 1, wherein the paper fiber of the base paper, in percent of oven-dry fiber, comprises:
  - 40 10–50 weight percent cellulose;
  - 45 15–60 weight percent wood pulp; and
  - 0–70 weight percent fiber from processed used-paper.
16. The printing paper according to claim 15, wherein said base paper comprises up to 18 weight percent mineral filler, in relation to oven-dry paper fiber.
17. The printing paper according to claim 1, wherein said base paper comprises at least 0.5 weight percent of a highly cationic starch.
18. The printing paper according to claim 17, wherein said starch content of said base paper is at least 1.3 weight percent.
19. The printing paper according to claim 1, wherein a mass surface density of the finished paper is from 40–80 g/m<sup>2</sup>.
20. The printing paper according to claim 19, wherein said mass surface density is from 50–65 g/m<sup>2</sup>.

\* \* \* \* \*